# EUROPEAN PATENT SPECIFICATION

(11) **EP 1 203 546 B1**
(45) Date of publication and mention of the grant of the patent: **17.05.2006**
(21) Application number: 01309328.1
(22) Date of filing: 02.11.2001
(51) Int. Cl.: A47C 27/12, A47C 27/00

(54) **Bed mattress filling materials**
Füllmaterial für Bettmatratze
Matière de remplissage pour un matelas de lit

(30) Priority: 02.11.2000 GB 0026804
(43) Date of publication of application: 08.05.2002
(73) Proprietor: John Cotton Group Limited, Mirfield, West Yorkshire WF14 0EH (GB)
(72) Inventor: Uttley, John Stewart, Hebden Bridge, West Yorkshire HX7 7EW (GB); Rushton, Carl, Bradford, West Yorkshire BD12 9LX (GB)
(74) Representative: Vaughan, Christopher Tammo

(56) References cited:
- EP-A- 1 067 227
- WO-A-99/16705
- JP-A- 57 161 149
- US-A- 4 100 324
- US-A- 4 260 660
- US-A- 5 586 350
- PATENT ABSTRACTS OF JAPAN vol. 1995, no. 02, 31 March 1995 (1995-03-31) & JP 06 327856 A (TOYOBO CO LTD), 29 November 1994 (1994-11-29)
- PATENT ABSTRACTS OF JAPAN vol. 018, no. 127 (M-1569), 2 March 1994 (1994-03-02) & JP 05 317541 A (REIICHIRO KAKEHASHI), 3 December 1993 (1993-12-03)

## Description

Textile fibre webs are widely used for bed mattress fillings to provide a structure which is both comfortable and resilient. To comply with fire safety requirements, the characteristics of the filling material must ensure resistance to smouldering and flaming ignition.

Many bed mattress fillings are produced either from a polyester staple fibre or from a cellulosic, usually cotton, fibre.

Polyester-based mattress fillings demonstrate good load bearing characteristics and are non-ignitable with smouldering cigarette and small flaming ignition sources. However, such fillings have a tendency to melt under the influence of an ignition source and thus may expose lower layers of the filling assembly to ignition.

Cotton based fillings have reduced load bearing characteristics but show an ability to absorb moisture (perspiration) and thereby provide a more comfortable sleeping surface. When subjected to an ignition source, cotton will char to form a protective barrier, but progressive smouldering of the cotton occurs. Conventionally, cotton materials are chemically treated to prevent smoulder and a common method is to apply approximately 10% by weight of boric acid powder.

It is known from WO 99/16705 to provide a non-woven blend of 20 to 100% polyester fibre and 0 to 80% cellulosic fibre. It is stated that the blend has improved thermal insulation and better moisture transport properties than pure polyester materials, but there is no discussion of ignition resistance. A similar blend of cotton and polyester fibres for use as a batting material is known from JP 57-161149, which is also silent as to ignition resistance.

An object of the present invention is to provide a blend of textile fibres for a bed mattress filling which improves fire safety performance without the need to apply fire-retardant chemicals but yet provides the comfort and load bearing characteristics of cellulosic and polymeric fibres.

According to the present invention there is provided use of a blend of cellulosic fibre and a polymeric fibre having a melting temperature lower than its temperature of decomposition for ensuring resistance to both shouldering and flaming ignition of a bed maitress fibre filling material including said blend, wherein the cellulosic fibre represents between 45wt% and 65wt% of the blend and the polymeric fibre represents between 35wt% and 55wt% of the blend, and wherein no fire retardant chemicals are used.

Preferably, the cellulosic fibre represents between 50wt% and 65wt% of the blend and the polymeric fibre represents between 35wt% and 50wt% of the blend.

An embodiment of the invention will now be described, by way of example only.

In accordance with the invention a textile fibre web for use as a bed mattress filling material, comprises a blend of polyester and cotton fibres. The web of fibres may be formed by any standard web forming technique for example carding and cross laying, air laying, straight laying, and may be provided as a non-bonded web, a chemically bonded web, a thermally bonded web or a mechanically bonded web, for example by needling.

Cotton rich blends are prone to smouldering ignition and polyester rich blends are prone to flaming ignition. A range of blend proportions is provided wherein smouldering ignition is prevented by polyester additions and flaming ignition is prevented by cotton additions. In broad terms this range is represented by between 45wt% and 65wt% cotton and between 33wt% and 55wt% polyester with the preferred range being from 50wt% to 65wt% cotton and from 35wt% to 50wt% polyester. The polyester fibres are typically 1.7 dtex to 50 dtex with a staple length of between 25mm and 100mm. The product weight range is typically from 50grams per square metre to 4,000 grams per square metre depending upon the intended use. For example, a lightweight filling at 300 grams per square metre may be used to provide a protective fire resistant cover or layer superimposed on less fire resistant materials where a web of 1,500 grams per square metre may be used.

Tests have shown that in these ranges, neither smouldering ignition nor flaming ignition will occur when a bed mattress containing the filling material is subject to ignition sources up to ignition source 5 (BS 5852) or its equivalent.

Two such tests are described in the following examples.

### Example 1

| | | |
|---|---|---|
| A blend of fibres of composition: | Polyester 17 dtex 60mm | 15wt% |
| | Cotton | 50wt% |
| | Polyester 4.4 dtex bicomponent | 35wt% |

was formed into a web using an air laying machine and was thermally bonded at a temperature of 160°C to produce a bonded web.

The product had a weight of 1200 g/m² and a thickness of approximately 60mm making it ideally suited for use as a bed mattress filling material.

A comparison of the blended filling with a filling consisting of 100wt% cotton is given in the following table.

| | 100wt% cotton | example product |
|---|---|---|
| weight (g/m²) | 1200 | 1200 |
| thickness (mm) | 38 | 58 |
| density (kg/m³) | 32 | 21 |
| Support @ 12500 Pa (mm) | 12 | 36 |
| Indentation @ 12500pa.(mm) | 26 | 22 |

The increased bulk (thickness) and the increased support demonstrate a significant increase in filling performance of the example product.

A bed mattress comprising a non-fire retardant insulator pad and the example product as a filling gave the following results when tested for ignitability.

### Fillings assembly

| | |
|---|---|
| UK - Furniture and Furnishings (Fire)(Safety) Regulations schedule 2 part 4 | no ignition |

### Bed Mattress

| | |
|---|---|
| BS EN 597 - 1 (cigarette test) | no ignition |
| BS EN 597 - 2 (match test) | no ignition |
| BS6807 ignition source 5 | no ignition |
| BS 7177 Low hazard (including ignition source (0/NS) | no ignition |

### Example 2

| | | |
|---|---|---|
| A blend of fibres of composition: | Polyester 7 dtex 60mm | 35wt% |
| | Cotton | 65wt% |

was formed into a non-bonded web by carding and cross lapping. The web was layered on to a paper carrier to assist handling. The non-bonded web had a weight of 300g/m².

The example product was used as the top layer in a bed mattress filling assembly and imparted non-ignitable properties to the fillings assembly and to the bed mattress as follows.

| | |
|---|---|
| BS EN 597 - 1 (cigarette test) | no ignition |
| BS EN 597 - 2 (match test) | no ignition |
| BS 6807 ignition source 5 | no ignition |
| BS 7177 low hazard (including ignition source 0/NS | no ignition |

It is not intended to limit the invention to the use of cotton and polyester. Other cellulosic fibres may be used such as viscose rayon. Also, any thermoplastic fibre may be used, which has a melting temperature lower than its temperature of decomposition.

Also, the filling may contain additional components representing no more than 20wt% of the overall blend. Examples are wool, PVC and some acrylics having a melting temperature greater than their temperature of decomposition. Such additional components could enhance the fire retardant properties of the product.

## Claims

1. Use of a blend of cellulosic fibre and a polymeric fibre having a melting temperature lower than its temperature of decomposition for ensuring resistance to both shouldering and flaming ignition of a bed maitress fibre filling material including said blend, wherein the cellulosic fibre represents between 45wt% and 65wt% of the blend and the polymeric fibre represents between 35wt% and 55wt% of the blend, and wherein no fire retardant chemicals are used.

2. Use according to Claim 1, wherein the cellulosic fibre represents between 50wt% and 65wt% of the blend and the polymeric fibre represents between 35wt% and 50wt% of the blend.

3. Use according to Claim 1 or Claim 2, wherein the cellulosic fibre is at least predominantly cotton.

4. Use according to any preceding claim, wherein the polymeric fibre is at least predominantly polyester.

5. Use according to Claim 4, wherein the polyester fibres included in the polymeric fibre proportion of the blend are in the range of 1.7 dtex to 50 dtex.

6. Use according to Claim 4 or 5, wherein the polyester fibres included in the polymeric content of the blend have a staple length of from 25mm to 100mm.

7. Use according to any preceding claim, wherein the material has a weight in the range of 50 grams per square metre to 4,000 grams per square metre.

8. Use according to any preceding claim, wherein additional components representing no more than 20wt% of the blend are added to the material.

9. Use according to Claim 8, wherein the additional components comprise one or more components selected from wool, PVC and acrylic materials having a melting temperature greater than their temperature of decomposition.

## Patentansprüche

1. Verwendung eines Mischgarns aus zellulosehaltiger Faser und einer Polymerfaser mit einer Schmelztemperatur unter seiner Zersetzungstemperatur zum Gewährleisten von Beständigkeit sowohl gegen Schwel- als auch Flammentzündung eines Bettmatratzenfaserfüllmaterials, das das Mischgarn umfasst, wobei die zellulosehaltige Faser zwischen 45 Gew.-% und 65 Gew.-% des Mischgarns darstellt und die Polymerfaser zwischen 35 Gew.-% und 55 Gew.-% des Mischgarns darstellt, und wobei keine feuerhemmenden Chemikalien verwendet sind.

2. Verwendung nach Anspruch 1, wobei die zellulosehaltige Faser zwischen 50 Gew.-% und 65 Gew.-% des Mischgarns darstellt und die Polymerfaser zwischen 35 Gew.-% und 50 Gew.-% des Mischgarns darstellt.

3. Verwendung nach Anspruch 1 oder 2, wobei die zellulosehaltige Faser zumindest vorwiegend Baumwolle ist.

4. Verwendung nach einem vorhergehenden Anspruch, wobei die Polymerfaser zumindest vorwiegend Polyester ist.

5. Verwendung nach Anspruch 4, wobei die Polyesterfasern, die in dem Polymerfaserverhältnis des Mischgarns umfasst sind, im Bereich von 1,7 dtex bis 50 dtex sind.

6. Verwendung nach Anspruch 4 oder 5, wobei die Polyesterfasern, die in dem Polymeranteil des Mischgarns umfasst sind, eine Stapellänge von 25 mm bis 100 mm aufweisen.

7. Verwendung nach einem vorhergehenden Anspruch, wobei das Material ein Gewicht im Bereich von 50 Gramm pro Quadratmeter bis 4.000 Gramm pro Quadratmeter aufweist.

8. Verwendung nach einem vorhergehenden Anspruch, wobei zusätzliche Komponenten, die nicht mehr als 20 Gew.-% des Mischgarns darstellen, zu dem Material hinzugefügt sind.

9. Verwendung nach Anspruch 8, wobei die zusätzlichen Komponenten eine oder mehrere Komponenten aufweisen, die aus Wolle, PVC und Acrylmaterialien mit einer Schmelztemperatur größer als ihre Zersetzungstemperatur ausgewählt sind.

## Revendications

1. Utilisation d'un mélange de fibres cellulosiques et de fibres polymères ayant une température de fusion inférieure à sa température de décomposition, pour assurer la résistance à la fois d'épaulement et d'allumage de flamme d'un matériau de remplissage à fibres pour matelas de lit, incluant ledit mélange, **caractérisée en ce que** la fibre cellulosique représente entre 45 % en poids et 65 % en poids du mélange, et la fibre polymère représente entre 35 % en poids et 55 % en poids du mélange, et **en ce qu'**aucun produit chimique retardateur de feu n'est utilisé.

2. Utilisation selon la revendication 1, **caractérisée en ce que** la fibre cellulosique représente entre 50 % en poids et 65 % en poids du mélange et la fibre polymère représente entre 35 % en poids et 50 % en poids du mélange.

3. Utilisation selon l'une des revendications 1 ou 2, **caractérisée en ce que** la fibre cellulosique est au moins de manière prédominante du coton.

4. Utilisation selon l'une des revendications précédentes, **caractérisée en ce que** la fibre polymère est au moins en prédominance du polyester.

5. Utilisation selon la revendication 4, **caractérisée en ce que** les fibres polyester incluses dans la proportion de fibres polymères du mélange sont dans la gamme de 1,7 dtex à 50 dtex.

6. Utilisation selon l'une des revendications 4 ou 5, **caractérisée en ce que** les fibres polyester incluses dans la teneur en polymères du mélange présentent une longueur de fibre entre 25 à 100 mm.

7. Utilisation selon l'une des revendications précédentes, **caractérisée en ce que** le matériau présente un poids dans la gamme de 50 g par mètre carré, et 4000g par mètre carré.

8. Utilisation selon l'une des revendications précédentes, **caractérisée en ce que** des composants additionnels ne représentant pas plus de 20 % en poids du mélange sont ajoutés au matériau.

9. Utilisation selon la revendication 8, **caractérisée en ce que** les composants additionnels comportent un ou plusieurs composants choisis parmi la laine, P. V. C., les matériaux acryliques, ayant une température de fusion plus grande que leur température de décomposition.
